

## UNITED STATES PATENT OFFICE

2,440,530

## STABILIZED ORGANIC COMPOSITIONS

Wallace J. Yates, Martinez, Calif., assignor to  
Shell Development Company, San Francisco,  
Calif., a corporation of Delaware

No Drawing. Application November 4, 1944,  
Serial No. 562,039

7 Claims. (Cl. 252—51.5)

1

This invention relates to compounded lubricating oil and to organic compositions possessing unusual oxidation stability and other desirable qualities due to the presence of the herein-described additives.

Organic compositions undergo oxidation upon exposure to air. This process is accentuated by increased temperature such as occurs in engines and other operating machinery. When such organic compositions are used as machinery lubricants, their stability is still further drastically reduced due to their contact with metal surfaces which give up metal into the lubricant. Such dissolved metals or metal salts act as oxidation catalysts in the lubricant and their action seems to be particularly drastic when both iron and copper are present. In addition, water also causes corrosion of metal parts and accentuates oxidation of the lubricant. Such water, even though not originally present in the oil, may come from a variety of sources such as condensation from the atmosphere due to changes in temperature, it may be formed by the oxidation of the lubricant, may enter by leakage into machinery used in aqueous or marine environments, etc.

A particular situation in which this problem of oxidation stability of an organic lubricant is especially serious is found in steam turbine lubricating systems. There the lubricant is exposed to high temperatures in the presence of iron, copper and water. The occurrence of rusting also contributes to the degradation of the oil and the rust may circulate through the oil system, interfere with clearances and clog delicate engine parts such as the governor mechanism. In addition, specifications for turbine lubricants require that the mineral oil base be highly refined and this, although it improves the lubricant in other respects, unfortunately tends to remove natural oxidation inhibitors from the oil. Further, since the prevention or minimization of emulsions is also an essential requirement in turbine operations, the use of many otherwise beneficial additives is precluded because of their tendency to contribute to emulsion formation.

Turbine oils can be produced, for example, from well refined lubricating oils of the proper viscosity range which may be about 75 to 750 Say. Univ. sec. at 100° F.

Similar problems of oxidation stability of lubricants used in contact with metal surfaces arise in connection with damping or hydraulic oils, transformer or electrical insulating oils, refrigerator oils, etc.

2

Further, application of the present addition agents is not limited to their use in hydrocarbon or mineral oil (petroleum) compositions but they may be employed similarly in lubricants composed in whole or in part of animal or vegetable ingredients such as natural waxes, sperm oil, whale oil, palm oil, jojoba oil, olive oil, Perilla oil, linseed oil, tung oil, soyabean oil, flaxseed oil, tallow, lard, stearine pitch, etc., as well as so-called synthetic lubricants such as polymerized olefins, alcohols, esters, etc.

Likewise, employment of the present additives is not limited to their use in lubricating compositions but they are broadly applicable to the stabilization of any organic compositions which are likely to come in contact with metal whether at elevated temperatures or not. They may be used generally in situations in which it is desired to inhibit both corrosion or rusting of a metal surface and oxidation of an organic composition which is in contact with such surface.

It is advantageous to apply to the present problem two additives—that is, an anticorrosive agent and an antioxidant—rather than try to make one additive perform both functions. A primary reason for this is that different amounts of the two types of ingredients are usually required. Also, since the anticorrosive agent generally functions by forming a film on the metal surface; if it were also employed as an antioxidant this film formation would withdraw it from the solution, thus diminishing the oxidation protection of the organic composition.

The corrosion or rust inhibitor used in the present combination is a relatively high molecular weight dibasic acid. By dibasic acid is meant an acid having two acidic or ionizable hydrogen ions. The two acidic radicals should be separated by no more than about four carbon atoms and preferably by no more than two or three. Such acids are, for instance, high molecular weight saturated or unsaturated polycarboxylic acids stable under ordinary lubricating conditions, such as alkylated aliphatic polycarboxylic acids like alkylated succinic, glutaric, adipic, etc., acids. The oxygen in the acid radicals may also be replaced in whole or in part by sulfur to give the corresponding thio equivalents as thionic (—COSH), thionic (—CSOH), or thionothionic (—CSSH) acids.

They may also be monocarboxylic acids whose second acidic hydrogen atom is supplied or activated by a radical such as hydroxyl, nitro, nitroso, cyano, hydrosulfide, or aromatic sulfonyl which is not more than about two or three carbon atoms

removed from the carboxylic radical. These monocarboxylic acids themselves should contain a minimum of 12 to 16 carbon atoms in addition to the added radical. Thus, taking stearic acid as an example, its dibasic corrosion-inhibiting derivatives would be alpha or beta hydroxystearic acid, alpha or beta nitrostearic acid, alpha or beta nitrosostearic acid, alpha or beta cyano-stearic acid, alpha or beta mercapto-stearic acid, alpha or beta phenylsulfonyl-stearic acid, etc.

One or both of the acidic groups may be attached to an aromatic nucleus, as in alkylated salicylic acid (e. g. di-isopropylsalicylic acid), alpha (orthocarboxyl aryloxy) carboxylic acids, e. g.



etc.

One may also use dibasic acids wherein the two acidic groups are joined through an oxygen, sulfide, disulfide or nitrogen linkage, as



wherein X is an oxygen, sulfur or nitrogen atom,  $y=0$  or 1,  $z$  is a small integer such as 1 or 2, and each R is an organic radical, conveniently a fatty acid radical.

Hydroxamic acids



are also effective dibasic corrosion inhibitors.

These corrosion inhibitors may also contain ether, amino, sulfide, disulfide, etc., radicals elsewhere in the molecule. Those dibasic acids having at least one carboxylic radical are preferred. Mixtures of the various dibasic acids, as well as the pure compounds, may be used.

The saturated acids are preferred because of their greater stability toward oxidation which results in longer active life. Also, these corrosion inhibitors consisting only of carbon, hydrogen and oxygen are preferred. The most useful and practical dibasic acids for the present purposes are alkylated succinic acids having a minimum of about 16 carbon atoms and preferably those having 20 or more carbon atoms. Suitable acids may be produced by taking olefins boiling above about 300° C., such as may be obtained by cracking paraffin wax or by dehydration of long chain fatty alcohols, etc., and condensing them with maleic acid anhydride to produce an alkylene succinic anhydride, hydrolyzing to produce the corresponding free acid which may then be hydrogenated if desired. Such acids have been described in U. S. Patent No. 2,133,734.

The second additive in the present combination is an oil-soluble organic compound in which two amino phenyl radicals are joined by no more than two atoms of carbon, nitrogen, oxygen, phosphorus, aluminum, boron, arsenic, antimony, or sulfur. The two atoms may be the same or different elements. These antioxidants thus have the basic formula



wherein X represents no more than two carbon, nitrogen, oxygen, phosphorus, aluminum, boron, arsenic, antimony or sulfur atoms. Those com-

pounds in which X is a carbon or sulfur atom or a disulfide group are preferred.

The amine groups may be primary, secondary or tertiary. Thus, the amino nitrogen atoms, as well as the phenyl nuclei may carry such low molecular weight alkyl radicals as methyl, ethyl, normal and isopropyl, n-, iso-, secondary-, and tertiary-butyl, amyl, hexyl, heptyl, octyl and higher homologs and isomers. When the 10 valences of X are not all taken by the two phenyl groups, the additional bonds may be occupied by like alkyl radicals, by hydrogen atoms, additional phenyl or aryl radicals, etc. Also, the phenyl radicals may, if desired, carry more than one 15 amino group. Thus, when X is a carbon atom, illustrative examples are tetramethyl diamino diphenyl methane, tetraethyl diamino diphenyl methane, tetramethyl triamino diphenyl methane, tetramethyl diamino triphenyl methane, tetraethyl diamino triphenyl methane, and the like. The alkyl, aryl, aralkyl, alkaryl, alicyclic or heterocyclic radical affixed to X, to the amino groups or to the phenyl nuclei may also have such substituents as halogen or sulfur, and like 20 radicals and substituents may also occur on the phenyl nucleus.

The described antioxidants in which X is mono- or di-sulfide may be illustrated by NN' 25 tetramethyl diamino diphenyl monosulfide, di-amino diphenyl disulfides, diamino dixylyl disulfides and higher homologues.

The unusual stability produced by the combination of small amounts of the present additives in a petroleum composition was demonstrated 30 by the turbine oil stability test described in 43 Proc. A. S. T. M. 275 (1943). This consists of subjecting the oil sample to a temperature of 95° C. in the presence of water, oxygen and an iron-copper catalyst, the time required to build up a 40 neutralization number of 2.0 mg. KOH/gm. oil being determined. The essential features of the test are as follows:

The oxidation cell is a glass tube 45 mm. x 600 mm. fitted with a mushroom water condenser 45 and an oxygen delivery tube with fritted glass outlet. The catalyst consists of lengths of No. 14 A. w. g. open-hearth iron wire and electrolytic copper wire, each three meters long and wound into coils about 0.625 in. in diameter. 50 The cell containing 300 ml. oil sample and the iron-copper catalyst is assembled with the condenser and oxygen inlet tube and placed in a thermostatically controlled bath capable of maintaining a temperature of 95±0.5° C. in the 55 sample. Oxygen is admitted at a rate of 3±0.5 liter per hour and at the end of 30 minutes, 60 ml. of distilled water is added to the cell. The test is then continued until acids are formed to the extent that the neutralization number of the 60 oil reaches a value of 2.0.

In this test a turbine oil, refined from California petroleum, had an oxidation life of approximately 100 hours by itself. Another sample of the same oil, to which had been added 0.01% w. of saturated alkyl succinic acid of approximately 370 molecular weight showed the same oxidation stability as the straight oil. A third sample of this turbine oil, to which had been added 0.2% w. of tetramethyl diamino diphenyl methane had 70 an oxidation life of 2500 hours. A fourth sample, however, which contained both 0.01% of the alkyl succinic acid and 0.2% of the tetramethyl diamino diphenyl methane exhibited an oxidation stability of around 6000 hours.

75 It will be noted that the corrosion inhibitor,

alkyl succinic acid, did not by itself appreciably affect the oxidation stability of the oil (although it inhibited rusting of the contingent metal surface), but, when the tetramethyl diamino diphenyl methane was present in addition, the oxidation life of the oil was more than double the expected additive effect which might be calculated from the result with each additive alone.

When the two are used together an adequate amount of both generally does not exceed a total of 0.25 to 1%. The corrosion-inhibiting dibasic acid should be present in a minimum of about 0.0025%, the polyamino polyphenyl compound in a minimum of about 0.01%. Usually a combined weight of 0.01 to 0.2% is satisfactory, although the combination of additives is not without effect even at much lower concentrations in a turbine or electrical insulating oil.

In some instances it may also be advantageous to incorporate an additional antioxidant in about the same proportions as the polyamino polyphenyl compound. The function of this supplemental antioxidant or third additive is to reinforce the primary antioxidant. This is desirable because different types of antioxidants seem to exhibit a maximum effectiveness in the presence of particular metal surfaces or metallic oxidation catalysts and a minimum effectiveness with other metals. Hence when several different metals are in contact with the lubricant, it is well to have antioxidants which are particularly effective toward two or more types of metals.

Two classes of supplemental antioxidants have been found especially advantageous in association with the present dibasic acid corrosion inhibitors and the polyamino polyphenyl antioxidants. The first class consists of the N-aryl naphthylamines, typified by phenyl alpha naphthylamine, phenyl beta naphthylamine and di-naphthylamines.

The second class consists of polyalkyl arylhydroxy compounds. That is, they may have only one hydroxyl group (alkyl phenols) or more than one hydroxyl group (alkyl cresol, alkyl resorcinol, etc.). Preferably short alkyl groups—having up to about eight or ten carbon atoms—are attached to the aromatic nucleus at the two, four and/or six positions; advantageously at least one of the alkyl radicals is a tertiary alkyl. Particular examples are ditertiary-butyl para-cresol, 2,4-dimethyl-6-tertiary octyl phenol, pentamethyl- or pentaethyl-phenol and tritertiary-butyl phenol.

Sulfur-containing antioxidants may also be present. These should have a minimum of about 10 carbon atoms. Such antioxidant sulfur may be in the form of mercaptans, as in decyl mercaptans, dodecyl mercaptans, cetyl mercaptans, oleyl mercaptans, stearyl mercaptans; butyl or other higher alkyl thiophenes; thionaphthols, alkyl thionaphthols, etc.; or of polysulfides

(R(SS)zR'

as in diamyl disulfide and higher dialkyl disulfides, e. g., diphenyl disulfides, dibenzyl disulfide, dinaphthyl disulfides, wax polysulfides formed by reaction of polychlorinated wax and sodium polysulfide, etc.); or of sulfur compounds formed by attaching sulfur to an olefinic double bond (as by reacting sulfur with olefins at temperatures of about 150° C. to 300° C.) which compounds are believed to contain the structure



(sulfur in epithio linkage).

Many sulfur compounds naturally occurring in petroleum oils are useful antioxidants, provided they have the proper reactivity. This may be determined by heating such compounds with finely divided metallic copper at 300° C. for 16 hours. Those compounds in which about 20% to 60% of the total sulfur content reacts with the copper under these conditions may be used as antioxidants.

10 Thiazoles such as mercaptobenzothiazole are also good antioxidants.

15 Among the sulfurized olefins found to be especially useful are, for example: sulfurized paraffin wax (as produced by chlorination of paraffin wax, having a molecular weight between about 225 and 425, dehydrochlorination of the chlorinated product to produce wax olefins, and sulfurization of the latter); sulfurized olefin or diolefin polymers boiling above about 400° C. such as obtained as by-products in the refining of cracked distillates with clay or other refining agents, or in the polymerization of normally gaseous olefins to produce gasoline or the like (e. g. sulfurized methyl pentadiene polymer); sulfurized esters of unsaturated fatty acids with monohydric alcohols, as methyl, ethyl, propyl, etc. oleate, or linoleate; sulfurized sperm oil; sulfurized jojoba oil; etc.

20 25 30 Also particularly effective are the oil-soluble reaction products of polychlor paraffin wax with sodium polysulfide which are compounds of the type



35 wherein  $n=2$  or more.

40 45 A compounded lubricating oil may also contain other additives like additional corrosion inhibitors, such as sulfonic or fatty acids and their salts, extreme pressure compounds such as alkyl phosphates, friction reducing compounds such as allophanates, interfacial tension modifiers or foam reducing agents, blooming agents, soap thickeners to form grease, viscosity regulators such as acryloid polymers, detergents, etc.

50 55 Detergents may be formed from the oil-soluble salts of various bases with detergent forming acids. Such bases include metallic as well as organic bases. Metallic bases include those of the alkali metals, as well as Cu, Mg, Ca, Sr, Ba, Zn, Cd, Al, Sn, Pb, Cr, Mn, Fe, Ni, Co, etc. Organic bases include various nitrogen bases as primary, secondary, tertiary and quaternary amines.

60 65 Examples of detergent forming acids are the various fatty acids of, say, 10 to 30 carbon atoms, wool fat acids, paraffin wax acids (produced by oxidation of paraffin wax), chlorinated fatty acids, aromatic carboxylic acids including aryl fatty acids, aryl hydroxy fatty acids, paraffin wax benzoic acids, various alkyl salicylic acids, phthalic acid mono esters, aromatic keto acids, aromatic ether acids; diphenols as di(alkyl phenol) sulfides and disulfides, methylene bis-alkyl-phenols; sulfonic acids such as may be produced by treatment of alkyl aromatic hydrocarbons or high boiling petroleum oils with sulfuric acid; sulfuric acid mono esters; phosphoric acid mono and di-esters, including the corresponding thiophosphoric acids, phosphonic and arsonic acids, etc.

70 Non-metallic detergents include compounds such as the phosphatides (e. g. lecithin), certain fatty oils as rapeseed oils, volatilized fatty or mineral oils.

75 Other detergents are the alkaline earth phos-

phate di-esters, including the thiophosphate di-esters; the alkaline earth diphenolates, specifically the calcium and barium salts of diphenol mono- and polysulfides; etc.

Particularly effective detergents are the polyvalent metal salts of the resinous condensation products of low molecular weight aldehydes (such as HCHO, CH<sub>3</sub>CHO, etc.) with alkylated aryl hydroxy products (such as alkyl phenol, alkyl naphthol, etc.). They may be typified by the calcium salt of the reaction product of formaldehyde and iso-octyl phenol



wherein *n* is a small integer such as 2, 3 or 4 or the product is a mixture of such polymers.

Detergents are employed in proportions of about 1/4% to about 5% weight.

The invention claimed is:

1. A refined mineral oil which is normally subjected to oxidative decomposition in the presence of a metal surface and containing a total of about 0.01% to 0.5% by weight of tetramethyldiamino diphenylmethane and a saturated alkyl succinic acid of at least 16 carbon atoms, the tetramethyldiamino diphenylmethane being present in a minimum amount of about 0.01% and the balance, not less than 0.0025% being a saturated alkyl succinic acid, the total amount not exceeding 0.5% by weight.

2. A mineral oil composition comprising a major proportion of a refined mineral oil which is normally subject to oxidative decomposition in the presence of a metal surface, a minimum amount of about 0.0025% of a saturated alkyl succinic acid of at least 16 carbon atoms and a minimum amount of about 0.01% of an N-alkylated diamino diphenylmethane, the total amount of the two additives not exceeding about 1.0% by weight.

3. A mineral oil composition comprising a major proportion of a mineral oil which is normally subject to oxidative decomposition in the presence of a metal surface, a minimum amount of about 0.0025% of an alkylated succinic acid of at least 16 carbon atoms and a minimum amount of about 0.01% of an N-alkylated diamino diphenylmethane, the total amount of the two additives not exceeding about 1.0% by weight.

4. An organic composition comprising a major proportion of a mineral oil which is normally subject to oxidative decomposition in the presence of a metal surface, a minimum amount of about 0.0025% of an alkylated succinic acid of at least 16 carbon atoms, and a minimum amount of

about 0.01% of tetramethyldiamino diphenylmethane, the total amount of the two additives not exceeding about 1.0% by weight and a minor amount of about 1.0% of an N-aryl naphthylamine.

5. An organic composition comprising a major proportion of a mineral oil which is normally subjected to oxidative decomposition in the presence of a metal surface, a minimum amount of about 0.0025% of a saturated alkyl succinic acid of at least 16 carbon atoms, and a minimum amount of about 0.01% of tetramethyldiamino diphenylmethane, the total amount of the two additives not exceeding about 1.0% by weight and a minor amount of about 1.0% of a polyalkylarylhydroxy compound.

6. An organic composition comprising a major proportion of a mineral oil which is normally subjected to oxidative decomposition in the presence of a metal surface, a minimum amount of about 0.0025% of a saturated alkyl succinic acid of at least 16 carbon atoms, and a minimum amount of about 0.01% of tetramethyldiamino diphenylmethane, the total amount of the two additives not exceeding about 1.0% by weight and a minor amount of about 1.0% of a phenyl alpha naphthylamine.

7. An organic composition comprising a major proportion of a mineral oil which is normally subjected to oxidative decomposition in the presence of a metal surface, a minimum amount of about 0.0025% of a saturated alkyl succinic acid of at least 16 carbon atoms and a minimum amount of about 0.01% of tetramethyldiamino diphenylmethane, the total amount of the two additives not exceeding about 1.0% by weight and a minor amount of about 1.0% of a diteriary-butyl-paracresol.

WALLACE J. YATES.

#### REFERENCES CITED

The following references are of record in the file of this patent:

#### UNITED STATES PATENTS

| Number    | Name      | Date          |
|-----------|-----------|---------------|
| 2,368,602 | Weiss     | Jan. 30, 1945 |
| 2,367,264 | Burk      | Jan. 16, 1945 |
| 2,366,074 | Wasson    | Dec. 26, 1944 |
| 2,350,746 | Fuller    | June 6, 1944  |
| 2,349,044 | Jahn      | May 16, 1944  |
| 2,346,356 | Burk      | Apr. 11, 1944 |
| 2,339,796 | Musher    | Jan. 25, 1944 |
| 2,334,158 | Von Fuchs | Nov. 9, 1943  |
| 2,290,860 | Burk      | July 28, 1942 |
| 2,220,723 | Lewis     | Nov. 5, 1940  |
| 2,202,877 | Stevens   | June 4, 1940  |
| 2,202,825 | Brandes   | June 4, 1940  |

**Certificate of Correction**

Patent No. 2,440,530.

April 27, 1948.

WALLACE J. YATES

It is hereby certified that error appears in the printed specification of the above numbered patent requiring correction as follows:

Column 3, lines 70 to 72 inclusive, for the formula



and that the said Letters Patent should be read with this correction therein that the same may conform to the record of the case in the Patent Office.

Signed and sealed this 8th day of March, A. D. 1949.

**[SEAL]**

**THOMAS F. MURPHY,**  
*Assistant Commissioner of Patents.*